# EUROPEAN PATENT APPLICATION

(11) **EP 4 632 145 A1**
(43) Date of publication of application: **15.10.2025**
(21) Application number: 24885702.1
(22) Date of filing: 29.10.2024
(51) Int. Cl.: D21H 17/04, C09K 3/18, D21H 11/12, D21H 21/14, D21H 21/16, D21H 27/10, D21J 5/00

(54) **PULP COMPOSITION**

(30) Priority: 01.11.2023 JP 2023187654
(71) Applicant: Daikin Industries, Ltd., Osaka-shi, Osaka 530-0001 (JP)
(72) Inventor: TANAKA, Asaka, Osaka-Shi, Osaka 530-0001 (JP); SHIBATA, Shun, Osaka-Shi, Osaka 530-0001 (JP); AKUTA, Ryo, Osaka-Shi, Osaka 530-0001 (JP)
(74) Representative: Hoffmann Eitle
(86) International application number: PCT/JP2024/038496
(87) International publication number: WO 2025/094934

(57) **Abstract**

Provided is a novel pulp composition comprising a wax and a pulp base material. The wax is a hydrocarbon wax, and the pulp base material contains bagasse pulp. The pulp composition has an oil-resistant property and/or a water-resistant property.

## Description

### Technical Field

The present disclosure relates to a pulp composition, and in particular to a pulp composition having oil resistance and/or water resistance.

### Background Art

Patent Literature 1 discloses that a composition containing sugar fatty acid ester and hemicellulose or lignin can be used to modify the barrier function of cellulose-based materials.

In the composition disclosed in Patent Literature 1, sugar fatty acid ester is an essential ingredient, and the use of other ingredients in place of sugar fatty acid ester has not been considered. Furthermore, Patent Literature 1 does not disclose that the composition exhibits excellent oil resistance and water resistance.

### Citation List

### Patent Literature

Patent Literature 1: WO 2021/019468

### Summary of Invention

### Technical Problem

An object of the present disclosure is to provide a novel pulp composition having oil resistance and/or water resistance.

### Solution to Problem

The present disclosure includes the following embodiments.

### [Item 1]

A pulp composition comprising a wax and a pulp substrate,
wherein
the wax is a hydrocarbon wax, and
the pulp substrate comprises bagasse pulp.

### [Item 2]

The pulp composition according to item 1, wherein the wax is at least one selected from the group consisting of paraffin wax and microcrystalline wax.

### [Item 3]

The pulp composition according to item 1 or 2, wherein the wax has a melting point of 40°C or more and 120°C or less.

### [Item 4]

The pulp composition according to any one of items 1 to 3, wherein an amount of the wax is 0.5% by weight or more and 25% by weight or less based on the pulp substrate.

### [Item 5]

The pulp composition according to any one of items 1 to 4, wherein an amount of the bagasse pulp is 20% by weight or more and 100% by weight or less in the pulp substrate.

### [Item 6]

The pulp composition according to any one of items 1 to 5, wherein the pulp composition comprises a dispersant.

### [Item 7]

The pulp composition according to any one of items 1 to 6, wherein the pulp composition comprises a combination chemical for paper.

### [Item 8]

The pulp composition according to any one of items 1 to 7, wherein the pulp composition comprises at least one selected from the group consisting of a sizing agent and a paper strength agent.

### [Item 9]

The pulp composition according to any one of items 1 to 8, wherein the pulp composition comprises aluminum sulfate.

### [Item 10]

A pulp formed article formed from the pulp composition according to any one of items 1 to 9.

### [Item 11]

The pulp formed article according to item 10, which is for food contact.

### [Item 12]

A method for producing a pulp composition, comprising treating a pulp substrate with a repellent comprising a wax, wherein
the wax is a hydrocarbon wax, and
the pulp substrate comprises bagasse pulp.

### [Item 13]

The method for producing a pulp composition according to item 12, wherein the wax is at least one selected from the group consisting of paraffin wax and microcrystalline wax.

### Advantageous Effect of Invention

The pulp composition of the present disclosure has excellent oil resistance and/or water resistance.

### Description of Embodiments

### <Pulp composition>

The pulp composition of the present disclosure comprises a wax and a pulp substrate. The pulp composition of the present disclosure has excellent oil resistance and/or water resistance, preferably both of the two.

The pulp composition of the present disclosure is obtained by adding a wax to a pulp substrate. The pulp composition may also be obtained by treating a pulp substrate with a repellent containing a wax. In that case the amount of the repellent added and the composition of the repellent may be adjusted so that the respective components are in desired amounts. The components in the repellent may also be separately added to the pulp composition as an additive.

The pulp composition of the present disclosure may not have any one selected from the group consisting of a compound having a fluoroalkyl group having 8 or more carbon atoms, a compound having a perfluoroalkyl group having 8 or more carbon atoms, a compound having a fluoroalkyl group having 4 or more carbon atoms, a compound having a perfluoroalkyl group having 4 or more carbon atoms, a compound having a perfluoroalkyl group, a compound having a fluoroalkyl group, and a compound having a fluorine atom. The pulp composition of the present disclosure can impart liquid-repellency to a substrate without including these fluorine-containing compounds.

The pulp composition may have a pH of 3 to 10, for example, 5 to 9, and in particular 6 to 8. The amount of the respective components may be adjusted to achieve such pH.

### {Pulp substrate}

The pulp composition comprises a pulp substrate. The pulp substrate is composed of pulp, which may be wood pulp, non-wood pulp, wastepaper pulp or the like, including at least bagasse pulp.

### [Wood pulp]

Wood pulp includes softwood kraft pulp from the genus Abies, Pinus and the like, and hardwood kraft pulp from the genus Acacia, Eucalyptus, Fagus, and Populus (e.g., poplar). Softwood kraft pulp includes, for example, unbleached softwood kraft pulp (NUKP), bleached softwood pulp (NBKP), semi-bleached softwood kraft pulp (NSBKP), and softwood sulfite pulp. Examples of hardwood kraft pulp include unbleached hardwood kraft pulp (LUKP), bleached hardwood kraft pulp (LBKP), semi-bleached hardwood kraft pulp (LSBKP), and hardwood sulfite pulp. The pulp may be used singly or in combination. Other than kraft pulp, in addition to softwood kraft pulp and hardwood kraft pulp, wood pulp includes stone ground pulp (SGP), pressurized stone ground pulp (PGW), refiner ground pulp (RGP), thermo-ground pulp (TGP), chemi-ground pulp (CGP), crushed wood pulp (GP), thermomechanical pulp (TMP), and other mechanical pulps. Furthermore, wastepaper pulp includes a disintegrated wastepaper pulp, a disintegrated and deinked wastepaper pulp or a disintegrated, deinked and bleached wastepaper pulp produced from brown waste paper, kraft envelope wastepaper, wastepaper of magazines, wastepaper of newspapers, wastepaper of flyers, sorted office paper, wastepaper of cardboard, hard white wastepaper, Kent wastepaper, wastepaper of poster paper and bond paper.

### [Non-wood pulp]

Examples of non-wood pulp include pulp prepared from bagass, kenaf, bamboo, linter, cotton, linen, hemp, ramie, straw, esparto, Manila hemp, Xyzal hemp, yellow hemp, flax, ganpi, paper bush and kozo (Japanese paper mulberry), and bagass, kenaf, bamboo and linter are preferred, and bagass is more preferred.

### [Fiber length of pulp]

The pulp has an average fiber length of preferably 0.1 mm or more, more preferably 0.3 mm or more and further preferably 0.5 mm or more from the viewpoint of the improvement in oil resistance, and preferably 5.0 mm or less, more preferably 4.0 mm or less, further preferably 3.0 mm or less, particularly preferably 2.0 mm or less, and most preferably 1.2 mm or less from the viewpoint of ease of manufacture.

### [Fiber width of pulp]

From the viewpoint of the improvement in oil resistance, the pulp has an average fiber width of preferably 5 µm or more, more preferably 10 µm or more, and further preferably 15 µm or more, and preferably 50 µm or less, more preferably 40 µm or less, and further preferably 30 µm or less.

### [Composition of pulp substrate]

The amount of bagasse pulp may be more than 0% by weight, 10% by weight or more, 20% by weight or more, 30% by weight or more, 40% by weight or more, 50% by weight or more, 60% by weight or more, or 70% by weight or more, and is preferably 20% by weight or more, and may be 100% by weight or less, 90% by weight or less, 80% by weight or less, 70% by weight or less, 60% by weight or less, 50% by weight or less, 40% by weight or less, 30% by weight or less, 20% by weight or less, or 10% by weight or less, and is for example, 80% by weight or less in the pulp substrate.

The total amount of pulp other than bagasse may be 0% by weight or more, 10% by weight or more, 20% by weight or more, 30% by weight or more, 40% by weight or more, 50% by weight or more, 60% by weight or more, or 70% by weight or more, and may be 99% by weight or less, 90% by weight or less, 80% by weight or less, 70% by weight or less, 60% by weight or less, 50% by weight or less, 40% by weight or less, 30% by weight or less, 20% by weight or less, or 10% by weight or less in the pulp substrate.

The amount of wood pulp may be 0% by weight or more, 10% by weight or more, 20% by weight or more, 30% by weight or more, 40% by weight or more, 50% by weight or more, 60% by weight or more, or 70% by weight or more, and 99% by weight or less, 90% by weight or less, 80% by weight or less, 70% by weight or less, 60% by weight or less, 50% by weight or less, 40% by weight or less, 30% by weight or less, 20% by weight or less, or 10% by weight or less in the pulp substrate.

### [Form of pulp substrate]

The form of the pulp substrate when the wax is added thereto may be, for example, pulp alone, pulp slurry, or a pulp product. Specific examples thereof include pulp, such as bleached or unbleached chemical pulp such as kraft pulp or sulfite pulp; bleached or unbleached high-yield pulp such as groundwood pulp, mechanical pulp, or thermomechanical pulp; pulp slurry including the above pulp; and a pulp product such as paper, a paper container and a pulp formed article.

### [Amount of pulp substrate]

The amount of pulp substrate may be 0.1% by weight or more, 0.5% by weight or more, 1% by weight or more, 3% by weight or more, 5% by weight or more, 10% by weight or more, 20% by weight or more, 30% by weight or more, 50% by weight or more, 75% by weight or more, or 90% by weight or more, and 99% by weight or less, 75% by weight or less, 50% by weight or less, 40% by weight or less, 30% by weight or less, 20% by weight or less, 10% by weight or less, 5% by weight or less, 4% by weight or less, or 3% by weight or less in the pulp composition. Typically, when the pulp composition is prepared by internal addition, the amount of pulp substrate is 30% by weight or less in the pulp composition; when the pulp composition is prepared by external addition, the amount of pulp substrate may be 75% by weight or more in the pulp composition.

The amount of the pulp substrate may be 50% by weight or more, 60% by weight or more, 70% by weight or more, 80% by weight or more, 90% by weight or more, 95% by weight or more, or 99% by weight or more, and 99.9% by weight or less, 95% by weight or less, 90% by weight or less, 85% by weight or less, 75% by weight or less, 65% by weight or less, or 55% by weight or less in the pulp composition excluding liquid medium.

### {Liquid medium}

The pulp composition may comprise a liquid medium. The liquid medium may be water, an organic solvent, or a mixture of water and an organic solvent. The liquid medium is typically an aqueous medium, and in particular, water. The liquid medium may comprise a liquid medium derived from repellent.

### [Amount of liquid medium]

The amount of the liquid medium may be 0.1% by weight or more, 0.5% by weight or more, 1% by weight or more, 3% by weight or more, 5% by weight or more, 10% by weight or more, 20% by weight or more, 30% by weight or more, 50% by weight or more, 75% by weight or more, 90% by weight or more, or 95% by weight or more, and 99% by weight or less, 75% by weight or less, 50% by weight or less, 40% by weight or less, 30% by weight or less, 20% by weight or less, 10% by weight or less, 5% by weight or less, 4% by weight or less, or 3% by weight or less in the pulp composition. Typically, when the pulp composition is prepared by internal addition, the amount of the liquid medium is 50% by weight or more, and in particular 90% by weight or more in the pulp composition; when the pulp composition is prepared by external addition, the amount of the liquid medium is 30% by weight or less, and in particular, 10% by weight or less in the pulp composition.

### {Wax}

The pulp composition comprises a wax, in particular hydrocarbon wax. Details of the types of the wax are the same as those of the wax in <Repellent>.

### [Amount of wax]

The amount of the wax may be 0.1% by weight or more, 0.3% by weight or more, 0.5% by weight or more, 0.75% by weight or more, 1.0% by weight or more, 2.0% by weight or more, or 3.0% by weight or more, and is preferably 0.5% by weight or more, and may be 25% by weight or less, 20% by weight or less, 15% by weight or less, 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less, and is for example 15% by weight or less, 5.0% by weight or less, or 3.0% by weight or less based on the pulp substrate.

The surface of the pulp substrate (for example, a pulp product such as paper, a paper container and a pulp formed article) may be externally treated with the wax. The amount of the wax included in the coating layer formed by the external addition treatment may be 0.01 g/m² or more, 0.03 g/m² or more, 0.05 g/m² or more, 0.1 g/m² or more, 0.3 g/m² or more, 0.5 g/m² or more, or 1.0 g/m² or more, and may be 5.0 g/m² or less, 4.0 g/m² or less, 3.0 g/m² or less, 2.0 g/m² or less, 1.0 g/m² or less, 0.5 g/m² or less, 0.3 g/m² or less, or 0.1 g/m² or less.

### {Dispersant}

The pulp composition may comprise a dispersant. Details of the types of the dispersant are the same as those of the dispersant in <Repellent>.

### [Amount of dispersant]

The amount of the dispersant may be 0.1% by weight or more, 0.3% by weight or more, 0.5% by weight or more, 0.75% by weight or more, 1.0% by weight or more, 2.0% by weight or more, or 3.0% by weight or more, and may be 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less, and is preferably 5.0% by weight or less, and more preferably 3.0% by weight or less based on the pulp substrate.

### {Paper strength agent}

The pulp composition may comprise a paper strength agent. Examples of paper strength agents include:
a polyacrylamide-based paper strength agent such as cationic polyacrylamide, anionic polyacrylamide and amphoteric polyacrylamide;
a polysaccharide-based paper strength agent such as starch, enzyme modified starch, thermochemically modified starch, oxidized starch, esterified starch, etherified starch (e.g., hydroxyethylated starch), aldehyde starch, cationized starch, starch, xanthan gum, gum karaya, welan gum, guar gum, pectin, tamarind gum, carrageenan, chitosan, gum arabic, locust bean gum, cellulose, alginic acid, agar, dextran, cellulose, carboxymethylcellulose, hydroxyethylcellulose, hydroxypropylcellulose, chitin nanofiber, cellulose nanofiber and pullulan, and a modified polysaccharide thereof (e.g., a modified polysaccharide prepared by introducing a hydroxyl group or a cationic group thereinto);
a polyamide-based paper strength agent such as polyamide resin, polyamine resin, polyamide-polyamine resin, polyamide-epichlorohydrin resin, polyamide-polyamine-epichlorohydrin resin, polyamide-polyurea-formaldehyde resin and epoxidized polyamide resin;
a urea/melamine paper strength agent such as urea resin, melamine resin, urea-formaldehyde resin and melamine-formaldehyde resin;
a polyvinyl alcohol paper strength agent such as polyvinyl alcohol, completely saponified polyvinyl alcohol, partially saponified polyvinyl alcohol, carboxyl modified polyvinyl alcohol, silanol modified polyvinyl alcohol, cation modified polyvinyl alcohol and terminal alkyl modified polyvinyl alcohol; and
a styrene butadiene copolymer, polyvinyl acetate, a vinyl chloride-vinyl acetate copolymer, polyvinyl chloride, polyvinylidene chloride, polyacrylic ester, fatty acid diamide, polyethyleneimine resin and ketone aldehyde resin.

A polyacrylamide-based paper strength agent, a polysaccharide-based paper strength agent and a polyamide-based paper strength agent are preferred as the paper strength agent in the present disclosure.

### [Amount of paper strength agent]

The amount of the paper strength agent may be 0.1% by weight or more, 0.3% by weight or more, 0.5% by weight or more, 0.75% by weight or more, 1.0% by weight or more, 2.0% by weight or more, or 3.0% by weight or more, and may be 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less, and is preferably 5.0% by weight or less based on the pulp.

### {Sizing agent}

The pulp composition may comprise a sizing agent. Examples of sizing agents include a cationic sizing agent, an anionic sizing agent, a neutral sizing agent and an amphoteric sizing agent, a rosin-based sizing agent (for example, an acidic rosin-based sizing agent and a neutral rosin-based sizing agent), alkyl ketene dimer and alkenyl succinic anhydride.

### [Amount of sizing agent]

The amount of the sizing agent may be 0.1% by weight or more, 0.2% by weight or more, 0.3% by weight or more, 0.5% by weight or more, 0.75% by weight or more, 1.0% by weight or more, 2.0% by weight or more, or 3.0% by weight or more, and may be 10% by weight or less, 7.5% by weight or less, 5.0% by weight or less, 4.0% by weight or less, 3.0% by weight or less, 2.0% by weight or less, 1.0% by weight or less, 0.75% by weight or less, or 0.5% by weight or less based on the pulp.

### {Other additives}

The pulp composition may also include another additive used for producing a pulp product in addition to the above components, including a known combination chemical for paper such as a fixing agent (e.g., aluminum sulfate), a coagulant and an agglomerating agent (e.g., polyamine-based resin), an yield improver (e.g., polyacrylamide-based resin), an organic acid (e.g., formic acid, acetic acid), a dye, a slime control agent, and an antifoaming agent.

### [Amount of other additives]

The amount of other additives may be 0.01% by weight or more, 0.1% by weight or more, 1% by weight or more, 3% by weight or more, 5% by weight or more, and may be 30% by weight or less, 20% by weight or less, 10% by weight or less, 5% by weight or less, 3% by weight or less, or 1% by weight or less, respectively, based on the pulp substrate.

### <Repellent>

The repellent in present disclosure adheres to a substrate (in particular, a pulp substrate) and imparts liquid-repellency, for example, water resistance, oil resistance, water-repellency, oil-repellency and/or antifouling properties to the substrate, and may function as a water-resistant agent, an oil-resistant agent, a water-repellent agent, an oil-repellent agent and/or an antifouling agent.

The repellent in the present disclosure includes a wax, in particular hydrocarbon-based wax, as the active ingredient. The wax itself may be used as a repellent, or may be combined with other components described below and used as a repellent.

The repellent of the present disclosure may not include one selected from the group consisting of a compound having a fluoroalkyl group having 8 or more carbon atoms, a compound having a perfluoroalkyl group having 8 or more carbon atoms, a compound having a fluoroalkyl group having 4 or more carbon atoms, a compound having a perfluoroalkyl group having 4 or more carbon atoms, a compound having a perfluoroalkyl group, a compound having a fluoroalkyl group and a compound having a fluorine atom. The repellent of the present disclosure can impart liquid-repellency to a substrate without these fluorine compounds.

The volume abundance ratio of particles with a size of 100 µm or larger in the repellent of the present disclosure may be 0.1% or more, 0.3% or more, 0.5% or more, 1% or more, 1.5% or more, 3% or more, 4% or more, 5% or more, or 10% or more, and may be 50% or less, 30% or less, 20% or less, 15% or less, 10% or less, 5% or less, 3% or less, or 1.5% or less, as measured by laser diffraction scattering. The method for setting the volume abundance ratio of particles with a size of 1 µm or larger as measured by laser diffraction scattering to the above range is not limited, and for example, particles in the raw material and/or dispersion may be formed into fine particles using a pulverizer or a homogenizer.

The volume median diameter of the repellent in the present disclosure as measured by laser diffraction scattering may be 0.01 µm or more, 0.05 µm or more, 0.1 µm or more, 0.2 µm or more, 0.3 µm or more, 0.4 µm or more, 0.5 µm or more, or 0.6 µm or more, and may be 10 µm or less, 5 µm or less, 3 µm or less, 1 µm or less, 0.9 µm or less, 0.8 µm or less, 0.7 µm or less, 0.6 µm or less, 0.5 µm or less, 0.4 µm or less, 0.3 µm or less, or 0.2 µm or less, and is preferably 1 µm or less. In the present disclosure, the volume median diameter refers to the median diameter (D50) in a volume-based particle size distribution by laser diffraction scattering.

The average particle size, obtained from an observation image by a scanning electron microscope, of the particle obtained by removing liquid medium from repellent (e.g., an oil resistant agent for pulp) which is the water-dispersible composition in the present disclosure by air dry at room temperature may be 0.01 µm or more, 0.05 µm or more, 0.1 µm or more, 0.2 µm or more, 0.3 µm or more, 0.4 µm or more, 0.5 µm or more, or 0.6 µm or more, and may be 10 µm or less, 5 µm or less, 3 µm or less, 1 µm or less, 0.9 µm or less, 0.8 µm or less, 0.7 µm or less, 0.6 µm or less, 0.5 µm or less, 0.4 µm or less, 0.3 µm or less, or 0.2 µm or less, and is preferably 1 µm or less. To set the particle size to the above range, for example, particles in the raw material and/or dispersion may be formed into fine particles using a pulverizer or a homogenizer. The room temperature means 20°C to 30°C, in particular 25°C.

The ionic charge density of the repellent in the present disclosure may be -1,000 µeq/g or more, -800 µeq/g or more, - 600 µeq/g or more, -500 µeq/g or more, -400 µeq/g or more, - 250 µeq/g or more, -100 µeq/g or more, -50 µeq/g or more, -25 µeq/g or more, 0 µeq/g or more, 1 µeq/g or more, 25 µeq/g or more, 50 µeq/g or more, 100 µeq/g or more, 200 µeq/g or more, and is preferably -600 µeq/g or more, and may be, for example, -400 µeq/g or more, -200 µeq/g or more, -50 µeq/g or more, and may be 5,000 µeq/g or less, 2,500 µeq/g or less, 1,000 µeq/g or less, 750 µeq/g or less, 500 µeq/g or less, 400 µeq/g or less, 350 µeq/g or less, 300 µeq/g or less, 200 µeq/g or less, 100 µeq/g or less, or 50 µeq/g or less, and is preferably 1,000 µeq/g or less, more preferably 500 µeq/g or less, and for example, 300 µeq/g or less. In particular, it is preferable that the repellent in the present disclosure has an ionic charge density of -600 µeq/g or more and 100 µeq/g or less. The ionic charge density of the repellent in the present disclosure may be measured by, for example, the following method.

The anion requirement of a sample solution having a solid content of 0.1 g/L is measured by a particle charge meter (MUTEK PCD-06 manufactured by BTG) using a 1/1,000 N potassium polyvinylsulfonate solution to calculate the ionic charge density (cationic charge density) by the following equation (1). Alternatively, the cation requirement is measured in the same manner by using poly(diallyldimethylammonium chloride) solution instead of the potassium polyvinylsulfonate solution to calculate the ionic charge density (anionic charge density) by the following equation (1). $Ionic charge density \left(μeq/g\right) = A / B$
A: cation requirement or anion requirement (µeq/L)
B: Concentration of sample solution (g/L)

### {Wax}

The repellent in the present disclosure comprises wax, in particular hydrocarbon wax. The wax may be an organic material that is solid at room temperature and liquid when heated. For example, the wax may be a hydrocarbon compound or a compound having a hydrocarbon group having 6 or more and 40 or less carbon atoms (e.g., an alkyl group).

The wax in the present disclosure adheres to a substrate (in particular, a pulp substrate) and imparts liquid repellency such as water resistance, oil resistance, water-repellency, oil-repellency and/or antifouling properties to the substrate.

### [Characteristics of wax]

Possible characteristics of the wax will be described below.

The wax may be in the form of particles (powder). The average particle size of the wax may be 0.01 µm or more, 0.05 µm or more, 0.1 µm or more, 0.2 µm or more, 0.3 µm or more, 0.4 µm or more, 0.5 µm or more, or 0.6 µm or more, and may be 10 µm or less, 5 µm or less, 3 µm or less, 1 µm or less, 0.9 µm or less, 0.8 µm or less, 0.7 µm or less, 0.6 µm or less, 0.5 µm or less, 0.4 µm or less, 0.3 µm or less, or 0.2 µm or less, and is preferably 1 µm or less. The above particle size is the primary particle size. The average particle size in the above range provides excellent particle stability and may improve liquid repellency. The average particle size may be measured by a microscope (scanning electron microscope). Specifically, a sample of wax particles is observed under a microscope at any magnification. Next, when the form of particles is spherical, the diameter is considered as the particle size, and when the form of particles is non-spherical, the average of the largest major axis and the largest minor axis is regarded as the particle size. By repeating measuring the particle size of all particles present in a field of view and moving to a different field of view and measuring the particle size again, 100 or more particle sizes are measured, and the average of those is defined as the average particle size.

The HD (n-hexadecane) contact angle of the wax may be 10° or more, 20° or more, 25° or more, 30° or more, 35° or more, 40° or more, 45° or more, 50° or more, 55° or more, 60° or more, or 65° or more, and is preferably 25° or more, more preferably 30° or more, and may be 100° or less, 90° or less, or 75° or less. A HD contact angle of the wax of the lower limit or more can impart good liquid-repellency (in particular oil-repellency) to a substrate. The HD contact angle is a static contact angle of the wax to a spin-coated film, which is obtained by dropping 2 µL of HD on a spin-coated film and measuring the contact angle one second after the droplet reaches the film.

The wax may have a water contact angle of 35° or more, 40° or more, 45° or more, 50° or more, 55° or more, 65° or more, 75° or more, 85° or more, 90° or more, or 100° or more, and may have 160° or less, 140° or less, 130° or less, 120° or less, 110° or less, 100° or less or 90° or less. A water contact angle of the wax of the lower limit or more can impart good liquid-repellency (in particular water-repellency) to a substrate. The water contact angle is a static contact angle of a wax to a spin-coated film, which is obtained by dropping 2 µL of water on a spin-coated film and measuring the contact angle one second after the droplet reaches the film.

The wax may be a low molecular weight compound (having a molecular weight of, for example, 1,000 or less or 500 or less) or a high molecular weight compound. When the wax is a high molecular weight compound, the wax may have a weight average molecular weight of 1,000 or more, 3,000 or more, 5,000 or more, 7,500 or more, 10,000 or more, 30,000 or more, 100,000 or more, 300,000 or more, or 500,000 or more, and 10,000,000 or less, 7,500,000 or less, 5,000,000 or less, 3,000,000 or less, 1,000,000 or less, 750,000 or less, 500,000 or less, 300,000 or less, 100,000 or less, 75,000 or less, 50,000 or less, 30,000 or less, 10,000 or less, 7,500 or less, 5,000 or less, or 3,000 or less.

The melting point of the wax may be 30°C or more, 40°C or more, 60°C or more, 80°C or more, 100°C or more, or 120°C or more, and is preferably 40°C or more, and may be 250°C or less, 225°C or less, 200°C or less, 150°C or less, 130°C or less, 120°C or less, 110°C or less, 100°C or less, 80°C or less, or 50°C or less, and is preferably 120°C or less. The melting point of wax may be measured according to JIS K 2235-1991.

### [Type of wax]

The wax in the present disclosure is a hydrocarbon wax. Examples thereof include petroleum wax such as paraffin wax, microcrystalline wax, montan wax, ozokerite wax, ceresin wax and petrolatum wax; and synthesized wax such as Fischer Tropsch wax, polyethylene wax and polypropylene wax, and paraffin wax and microcrystalline wax are preferred.

### [Amount of wax]

The amount of wax may be 0.01% by weight or more, 0.5% by weight or more, 1% by weight or more, 3% by weight or more, 5% by weight or more, 10% by weight or more, 20% by weight or more, 30% by weight or more, 50% by weight or more, 70% by weight or more, or 80% by weight or more, and may be 95% by weight or less, 90% by weight or less, 80% by weight or less, 70% by weight or less, 60% by weight or less, 50% by weight or less, 40% by weight or less, 30% by weight or less, 20% by weight or less, 10% by weight or less, 5% by weight or less, or 3% by weight or less in the repellent. Wax may be singly used as a repellent.

### {Dispersant}

The repellent in the present disclosure may comprise a dispersant. The dispersant may be at least one selected from an organic dispersant and an inorganic dispersant. The dispersant may be at least one selected from an anionic dispersant, a nonionic dispersant, a cationic dispersant, an amphoteric dispersant and an inorganic dispersant.

An organic dispersant and an inorganic dispersant may be used as the dispersant, respectively, or an organic dispersant and an inorganic dispersant may be used in combination.

An organic dispersant may be used as the dispersant. The organic dispersant may be classified into a nonionic dispersant, an anionic dispersant, a cationic dispersant and an amphoteric dispersant. The organic dispersant may mean a surfactant.

The dispersant may have no fluorine.

### [Nonionic dispersant]

The dispersant may comprise a nonionic dispersant. The nonionic dispersant may be a nonionic surfactant.

The nonionic dispersant may be of low molecular weight or high molecular weight. The nonionic dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of nonionic dispersant include ether, ester, ester ether, alkanolamide, polyol and amine oxide.

The ether is, for example, a compound having an oxyalkylene group (preferably a polyoxyethylene group).

The ester is, for example, an ester of an alcohol and a fatty acid. The alcohol is, for example, an alcohol which is 1 to 30 hydric (particularly dihydric to decahydric) and has 1 to 50 carbon atoms (particularly 10 to 30 carbon atoms) (for example, an aliphatic alcohol). Examples of the fatty acids are saturated or unsaturated fatty acids having 2 to 50 carbon atoms, particularly 5 to 30 carbon atoms.

The ester ether is, for example, a compound in which an alkylene oxide (particularly ethylene oxide) is added to an ester of an alcohol and a fatty acid. The alcohol is, for example, an alcohol which is 1 to 30 hydric (particularly dihydric to decahydric) and has 1 to 50 carbon atoms (particularly 3 to 30 carbon atoms) (for example, an aliphatic alcohol). Examples of the fatty acids are saturated or unsaturated fatty acids having 2 to 50 carbon atoms, particularly 5 to 30 carbon atoms.

The alkanolamide is formed of for example, a fatty acid and an alkanolamine. The alkanolamide may be a monoalkanolamide or a dialkanolamide. Examples of the fatty acids are saturated or unsaturated fatty acids having 2 to 50 carbon atoms, particularly 5 to 30 carbon atoms. The alkanolamine may be an alkanol with 1 to 3 amino groups and 1 to 5 hydroxyl groups, having 2 to 50, particularly 5 to 30 carbon atoms.

The polyol may be, for example, a dihydric to pentahydric alcohol having 10 to 30 carbon atoms.

The amine oxide may be an oxide (for example, having 5 to 50 carbon atoms) of an amine (secondary amine or preferably tertiary amine).

The nonionic dispersant is preferably a nonionic dispersant having an oxyalkylene group (preferably a polyoxyethylene group). The alkylene group in the oxyalkylene group preferably has 2 to 10 carbon atoms. The number of oxyalkylene groups in the molecule of the nonionic dispersant is generally preferably 2 to 100.

The nonionic dispersant is selected from the group consisting of an ether, an ester, an ester ether, an alkanolamide, a polyol, or an amine oxide, and is preferably a nonionic dispersant having an oxyalkylene group.

The nonionic dispersant may be, for example, an alkylene oxide adduct of a linear and/or branched aliphatic (saturated and/or unsaturated) group, a polyalkylene glycol ester of a linear and/or branched fatty acid (saturated and/or unsaturated), a sorbitan ester of a linear and/or branched fatty acid (saturated and/or unsaturated), a glycerin ester of a linear and/or branched fatty acid (saturated and/or unsaturated), a polyglycerol ester of a linear and/or branched fatty acid (saturated and/or unsaturated), a sucrose ester of a linear and/or branched fatty acid (saturated and/or unsaturated), a polyoxyethylene (POE)/polyoxypropylene (POP) copolymer (random copolymer or block copolymer), and an alkylene oxide adduct of acetylene glycol. Among them, the nonionic dispersant is preferably a dispersant such that the structures of the alkylene oxide addition moiety and polyalkylene glycol moiety are polyoxyethylene (POE) or polyoxypropylene (POP) or POE/POP copolymer (which may be a random or block copolymer, for example.).

Furthermore, the nonionic dispersant may not include an aromatic group.

The nonionic dispersant may be the compound represented by the formula:

R¹O-(CH₂CH₂O)ₚ-(R²O)_{q}-R³

[wherein R¹ is an alkyl group having 1 to 22 carbon atoms, an alkenyl group or an acyl group, having 2 to 22 carbon atoms, R² is each independently the same or different and is an alkylene group having 3 or more carbon atoms (for example, 3 to 10),
R³ is a hydrogen atom, an alkyl group having 1 to 22 carbon atoms, or an alkenyl group having 2 to 22 carbon atoms,
p is a numeral of 2 or more,
q is 0 or a numeral of 1 or more.].

R¹ preferably has 8 to 20 carbon atoms, particularly 10 to 18 carbon atoms. Preferred examples of R¹ include an octyl group, a nonyl group, a trimethylnonyl group, a lauryl group, a tridecyl group, an oleyl group and a stearyl group.

R² is, for example, a propylene group and a butylene group.

In the nonionic dispersant, for example, p may be a numeral of 3 or more (for example, 5 to 200) and q may be a numeral of 2 or more (for example, 5 to 200). Namely, -(R²O)_{q}-may form, for example, a polyoxyalkylene chain.

The nonionic dispersant may be, for example, a polyoxyethylene alkylene alkyl ether comprising a hydrophilic polyoxyethylene chain and a hydrophobic oxyalkylene chain (particularly a polyoxyalkylene chain) in the center. The hydrophobic oxyalkylene chain includes, for example, an oxypropylene chain, an oxybutylene chain, and a styrene chain. The oxypropylene chain is preferred among them.

Specific examples of the nonionic dispersants include a condensation product of ethylene oxide with hexylphenol, isooctatylphenol, hexadecanol, oleic acid, an alkane(C₁₂-C₁₆)thiol, a sorbitan monofatty acid (C₇-C₁₉), an alkyl (C₁₂-C₁₈)amine, or the like, and a sorbitan fatty acid ester, a glycerin fatty acid ester, a polyglycerin fatty acid ester, a sucrose fatty acid ester, a propylene glycol fatty acid ester, a polyoxyethylene alkyl ether, a polyoxyethylene polyoxypropylene alkyl ether, a polyoxyethylene glycerin fatty acid ester, a polyoxyethylene sorbitan fatty acid ester, and a lecithin derivative. Examples of nonionic dispersants include polyoxyethylene alkyl ether, polyoxyethylene polyoxypropylene alkyl ether, polyoxyethylene polyoxybutylene alkyl ether, polyoxyethylene polyoxypropylene glycol and polyethyleneimine ethoxylate.

The proportion of the polyoxyethylene block can be 5 to 80% by weight, for example, 30 to 75% by weight, particularly 40 to 70% by weight, based on a molecular weight of the nonionic dispersant (copolymer).

The average molecular weight of the nonionic dispersant is generally 300 to 5,000, for example, 500 to 3,000.

For example, the nonionic dispersant may be used singly or in admixture of two or more. The nonionic dispersant may be a mixture of a compound with an HLB (hydrophilic-hydrophobic balance) of less than 15 (particularly 5 or less) and a compound with an HLB of 15 or more. More specifically, it is preferable to select the nonionic dispersant from polyoxyethylene alkyl ether, polyoxyethylene polyoxypropylene alkyl ether, polyoxyethylene and polyoxypropylene having an HLB of 1 to 18, sorbitan fatty acid ester, glycerol fatty acid ester, polyglycerol fatty acid ester, sucrose fatty acid ester, propylene glycol fatty acid ester, polyoxyethylene glycerol fatty acid ester and polyoxyethylene sorbitan fatty acid ester having an HLB of less than 7.

### [Cationic dispersant]

The dispersant may comprise a cationic dispersant. The cationic dispersant may be a cationic surfactant. The cationic dispersant may be a compound not having an amide group.

The cationic dispersant may be of low molecular weight (with a molecular weight of 2,000 or less, in particular, 10,000 or less) or of high molecular weight (with a molecular weight of, for example, 2,000 or more). The cationic dispersant may not have an amide group. The cationic dispersant may have a molecular weight of 100 or more, 500 or more, 1,000 or more, 2,000 or more, 4,000 or more, or 6,000 or more, and 1,000,000 or less, 750,000 or less, 500,000 or less, 250,000 or less, 100,000 or less, 50,000 or less, 10,000 or less, 7,500 or less, 5,000 or less, 25,000 or less, 750 or less, or 250 or less.

The cationic dispersant may be aliphatic or aromatic, and examples thereof include an ammonium salt (e.g., quaternary ammonium salt). The cationic dispersant may be oxyethylene-added ammonium salt. Specific examples thereof include an amine salt dispersant such as alkylamine salt, an amino alcohol fatty acid derivative, a polyamine fatty acid derivative and imidazoline; a quaternary ammonium salt dispersant such as alkyl trimethyl ammonium salt, dialkyl dimethyl ammonium salt, alkyl dimethyl benzyl ammonium salt, pyridinium salt, alkyl isoquinolinium salt, benzalkonium chloride and benzethonium chloride; and a polymer cationic dispersant such as polyquaternium-1 to 47. Examples of cationic dispersants include alkyl amine salt and quaternary ammonium salt.

The low molecular weight cationic dispersant may be a compound represented by the formula:

R²¹-N⁺(-R²²)(-R²³)(-R²⁴)X⁻

wherein R²¹, R²², R²³ and R²⁴ are a hydrogen or a hydrocarbon group having 1 to 40 carbon atoms, and
X is an anionic group. Specific examples of R²¹, R²², R²³ and -R²⁴ include an alkyl group (e.g., a methyl group, a butyl group, a stearyl group, a palmityl group) and an aromatic group (e.g., a benzyl group, phenyl group). Specific examples of X include a halogen (e.g., chlorine) and an acid (e.g., hydrochloric acid and acetic acid). The cationic dispersant may be monoalkyltrimethylammonium salt (in which alkyl has 4 to 40 carbon atoms) and benzalkonium chloride.

More specifically, the low molecular weight cationic dispersant may be an ammonium salt represented by the formula:

R¹ₚ-N⁺-R²_{q}X⁻

[wherein R¹ is a C12 or higher (e.g., C₁₂ to C₅₀) linear and/or branched aliphatic (saturated and/or unsaturated) group,
R² is H or a C1 to 4 alkyl group, a benzyl group, a polyoxyethylene group (in which the number of oxyethylene groups is for example, 1 (in particular 2, and especially 3) to 50) (particularly preferably CH₃, C₂H₅),
X is a halogen atom (e.g., chlorine) or a C₁ to C₄ fatty acid salt or a C₁ to C₄ sulfonate,
p is 1 or 2, q is 2 or 3 and p + q = 4.]
R¹ may have 12 to 50, and for example 12 to 30 carbon atoms.

Examples of the low molecular weight cationic dispersants may include dodecyltrimethylammonium acetate, trimethyltetradecylammonium chloride, hexadecyltrimethylammonium bromide, trimethyloctadecylammonium chloride, (dodecylmethylbenzyl)trimethylammonium chloride, benzyldodecyldimethylammonium chloride, methyldodecyl di(hydropolyoxyethylene) ammonium chloride, benzyldodecyl di(hydropolyoxyethylene) ammonium chloride, and N-[2-(diethylamino)ethyl]oleamide hydrochloride.

The high molecular weight cationic dispersant may be a polymer having a cationic group (for example, an ammonium group, a quaternary ammonium group) (for example, polypolyquaternium-1 to 47). Examples of high molecular weight cationic dispersants include a cationic natural product (in particular, cationic sugar) such as cationic starch, cationic cellulose (e.g., O-(2-hydroxy-3-(trimethylammonio)propyl)hydroxyethyl cellulose chloride), cationic guar gum, cationic xanthan gum and chitosan; a polymer of a cationic group-containing monomer such as aziridine, vinyl imidazole, aminoalkyl methacrylate, N,N,N',N'-tetramethyl-2-butene-1,4-diamine, quaternary dimethyl ammonium ethyl methacrylic acid, diallyldimethylammonium chloride, dimethylaminopropylamine and quaternary vinyl imidazole.

### [Anionic dispersant]

The dispersant may comprise an anionic dispersant. The anionic dispersant may be an anionic surfactant. The dispersant may not include an anionic dispersant.

The anionic dispersant may be of low molecular weight or high molecular weight. The anionic dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of the anionic dispersant include an alkyl ether sulfate, an alkyl sulfate, an alkenyl ether sulfate, an alkenyl sulfate, an olefin sulfonate, an alkanesulfonate, a saturated or unsaturated fatty acid salt, an alkyl or alkenyl ether carbonate, an α-sulfone fatty acid salt, a N-acylamino acid dispersant, a phosphate mono- or diester dispersant, and a sulfosuccinic acid ester. Examples of anionic dispersants include a carboxylic acid salt (e.g., fatty acid salt).

### [Amphoteric dispersant]

The dispersant may comprise an amphoteric dispersant. The amphoteric dispersant may be an amphoteric surfactant.

The amphoteric dispersant may be of low molecular weight or high molecular weight. The amphoteric dispersant may have a molecular weight of 100 or more, 500 or more, 1,000 or more, 2,000 or more, 4,000 or more, or 6,000 or more, and 100,000 or less, 10,000 or less, 7,500 or less, 5,000 or less, 25,000 or less, 750 or less, or 250 or less.

Examples of the amphoteric dispersants include, for example, alanines, imidazolinium betaines, amidobetaines, and acetic acid betaine, and specific examples of the amphoteric dispersants include, for example, lauryl betaine, stearyl betaine, lauryl carboxymethyl hydroxyethyl imidazolinium betaine, lauryl dimethylamino acetic acid betaine, and fatty acid amidopropyldimethylaminoacetic acid betaine.

### [Inorganic dispersant]

The dispersant may comprise an inorganic dispersant.

The inorganic dispersant has an average primary particle size of 5 nm or larger, 30 nm or larger, 100 nm or larger, 1 µm or larger, 10 µm or larger, or 25 µm or larger, and 100 µm or smaller, 50 µm or smaller, 10 µm or smaller, 1 µm or smaller, 500 nm or smaller, or 300 nm or smaller. The average primary particle size may be measured by a microscope, for example, a scanning electron microscope or a transmission electron microscope. The inorganic dispersant may be hydrophilic particles.

Examples of inorganic dispersants include polyvalent metal phosphate such as tricalcium phosphate, magnesium phosphate, aluminum phosphate, zinc phosphate and hydroxyapatite; carbonate such as calcium carbonate and magnesium carbonate; silicate such as calcium metasilicate; sulfate such as calcium sulfate and barium sulfate; and hydroxide such as calcium hydroxide, magnesium hydroxide and aluminum hydroxide.

### [Amount of Dispersant]

The amount of dispersant may be 0.01 parts by weight or more, 0.1 parts by weight or more, 1 part by weight or more, 3 parts by weight or more, 5 parts by weight or more, 10 parts by weight, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less 30 parts by weight or less, 20 parts by weight or less, 10 parts by weight or less, 5 parts by weight or less, 3 parts by weight or less, or 1 part by weight or less.

### {Liquid medium}

The repellent in the present disclosure may comprise a liquid medium. The liquid medium may be water, an organic solvent, or a mixture of water and an organic solvent. The repellent may be a dispersion or a solution. The repellent in the present disclosure may include at least water.

Examples of the organic solvents include esters (for example, esters having 2 to 40 carbon atoms, specifically ethyl acetate and butyl acetate), ketones (for example, ketones having 2 to 40 carbon atoms, specifically methyl ethyl ketone and diisobutyl ketone), alcohols (for example, alcohols having 1 to 40 carbon atoms, specifically isopropyl alcohol), aromatic solvents (for example, toluene and xylene), petroleum-based solvents (for example, alkanes having 5 to 10 carbon atoms, specifically, naphtha and kerosene). The organic solvent is preferably a water-soluble organic solvent. The water-soluble organic solvent may include a compound having at least one hydroxy group (for example, polyol such as alcohol and glycol solvent, and an ether form of polyol (for example, a monoether form)). These may be used alone, or two or more of them may be used in combination.

### [Amount of liquid medium]

The amount of liquid medium may be 1 part by weight or more, 3 parts by weight or more, 5 parts by weight or more, 10 parts by weight or more, 20 parts by weight or more, 30 parts by weight or more, 40 parts by weight or more, or 50 parts by weight or more, 100 parts by weight or more, 200 parts by weight or more, 300 parts by weight or more, 500 parts by weight or more, or 1,000 parts by weight or more, and may be 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less relative to 1 part by weight of the wax.

The amount of water may be 1 part by weight or more, 3 parts by weight or more, 5 parts by weight or more, 10 parts by weight or more, 20 parts by weight or more, 30 parts by weight or more, 40 parts by weight or more, 50 parts by weight or more, 100 parts by weight or more, 200 parts by weight or more, 300 parts by weight or more, 500 parts by weight or more, or 1,000 parts by weight or more, and may be 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less based on 1 part by weight of the wax.

The amount of the organic solvent may be 1 part by weight or more, 3 parts by weight or more, 5 parts by weight or more, 10 parts by weight or more, 20 parts by weight or more, 30 parts by weight or more, 40 parts by weight or more, 50 parts by weight or more, 100 parts by weight or more, 200 parts by weight or more, 300 parts by weight or more, 500 parts by weight or more, or 1,000 parts by weight or more, and may be 3,000 parts by weight or less, 2,000 parts by weight or less, 1,000 parts by weight or less, 500 parts by weight or less, 200 parts by weight or less, 175 parts by weight or less, 150 parts by weight or less, 125 parts by weight or less, 100 parts by weight or less, 80 parts by weight or less, 60 parts by weight or less, 40 parts by weight or less, 20 parts by weight or less, or 10 parts by weight or less relative to 1 part by weight of the wax.

### {Silicone}

The repellent in the present disclosure may include silicone (polyorganosiloxane). Containing the silicone enables providing favorable texture and durability in addition to favorable liquid-repellency.

As the silicone, a known silicone can be used, and examples of the silicone include a polydimethylsiloxane and modified silicones (for example, amino-modified silicone, epoxy-modified silicone, carboxy-modified silicone, and methylhydrogen silicone). For example, the silicone may be silicone wax having waxy properties. These may be used singly or in combination of two or more thereof.

A weight average molecular weight of the silicone may be 1,000 or more, 10,000 or more, or 50,000 or more, and may be 500,000 or less, 2,500,000 or less, 100,000 or less, or 50,000 or less.

### [Amount of Silicone]

The amount of silicone may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less.

### {Organic Acid}

The repellent of the present disclosure may contain an organic acid. As the organic acid, a known organic acid can be used. Examples of the organic acid preferably include, for example, a carboxylic acid, a sulfonic acid, and a sulfinic acid, with the carboxylic acid being particularly preferred. Examples of the carboxylic acid include, for example, formic acid, acetic acid, propionic acid, butyric acid, oxalic acid, succinic acid, glutaric acid, adipic acid, malic acid, and citric acid, with the formic acid or acetic acid being particularly preferred. In the present disclosure, one type of organic acid may be used, or two or more thereof may be combined for use. For example, formic acid and acetic acid may be combined for use.

### [Amount of Organic Acid]

The amount of organic acid may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less. The amount of organic acid may be adjusted so that a pH of the repellent is 3 to 10, for example 5 to 9, particularly 6 to 8. For example, the repellent may be acidic (pH of 7 or less, for example 6 or less).

### {Inorganic acid}

The repellent in the present disclosure may comprise an inorganic acid. As the inorganic acid, a known inorganic acid can be used. Examples of inorganic acids include hydrogen chloride, hydrogen bromide, hydrogen iodide, nitric acid, boric acid, sulfuric acid and phosphoric acid. In the present disclosure, one inorganic acid may be used, or two or more of them may be used in combination. The addition of inorganic acid can improve the stability of the aqueous dispersion.

### [Amount of inorganic acid]

The amount of the inorganic acid may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less based on 100 parts by weight of the wax. The amount of the inorganic acid may be adjusted so that the repellent has a pH of 3 to 10, for example, 5 to 9, and in particular, 6 to 8. The repellent may be acidic (may have a pH of 7 or less, for example, 6 or less).

### {Curing Agent}

The repellent of the present disclosure may contain a curing agent (active hydrogen-reactive compound or active hydrogen-containing compound).

The curing agent (cross-linking agent) in the repellent can effectively cure the repellent. The curing agent may be an active hydrogen-reactive compound or an active hydrogen-containing compound, which reacts with an active hydrogen or an active hydrogen-reactive group. Examples of the active hydrogen-reactive compound include an isocyanate compound, epoxy compound, chloromethyl group-containing compound, carboxyl group-containing compound, and hydrazide compound. Examples of the active hydrogen-containing compound include a hydroxyl group-containing compound, an amino group-containing compound and a carboxyl group-containing compound, a ketone group-containing compound, a hydrazide compound, and a melamine compound.

The curing agent may contain an isocyanate compound. The isocyanate compound may be a polyisocyanate compound. The polyisocyanate compound is a compound having two or more isocyanate groups in one molecule. The polyisocyanate compound serves as a cross-linking agent. Examples of the polyisocyanate compound include, for example, an aliphatic polyisocyanate, an alicyclic polyisocyanate, an araliphatic polyisocyanate, an aromatic polyisocyanate, and derivatives of these polyisocyanates. The isocyanate compound may be a blocked isocyanate compound (for example, a blocked polyisocyanate compound). The blocked isocyanate compound is a compound in which an isocyanate group of an isocyanate compound is masked with a blocking agent to inhibit reaction.

Examples of the aliphatic polyisocyanates are aliphatic triisocyanates such as trimethylene diisocyanate, tetramethylene diisocyanate, hexamethylene diisocyanate, pentamethylene diisocyanate, 1,2-propylene diisocyanate, 1,2-butylene diisocyanate, 2,3-butylene diisocyanate, 1,3-butylene diisocyanate, 2,4,4- or 2,2,4-trimethylhexamethylene diisocyanate, an aliphatic diisocyanate of 2,6-diisocyanatomethylcaproate, and aliphatic triisocyanates such as lysine ester triisocyanate, 1,4,8-triisocyanateoctane, 1,6,11-triisocyanatoundecane, 1,8-diisocyanato-4-isocyanatomethyloctane, 1,3,6-triisocyanatohexane, 2,5,7-trimethyl-1,8-diisocyanato-5-isocyanatomethyloctane. These may be used singly or in combination of two or more thereof.

Examples of the alicyclic polyisocyanates include, for example, an alicyclic diisocyanate and an alicyclic triisocyanate. Specific examples of the alicyclic polyisocyanate include 1,3-cyclopentene diisocyanate, 3-isocyanatomethyl-3,5,5-trimethylcyclohexyl isocyanate (isophorone diisocyanate), and 1,3,5-triisocyanatocyclohexane. These may be used singly or in combination of two or more thereof.

Examples of the aromatic-aliphatic polyisocyanate include an aromatic-aliphatic diisocyanate and aromatic-aliphatic triisocyanate. Specific examples of the araliphatic polyisocyanate include 1,3- or 1,4-xylylene diisocyanate or a mixture thereof, 1,3- or 1,4-bis(1-isocyanato-1-methylethyl)benzene (tetramethyl xylylene diisocyanate) or a mixture thereof, and 1,3,5-triisocyanatomethylbenzene. These may be used singly or in combination of two or more thereof.

Examples of the aromatic polyisocyanates include an aromatic diisocyanate, aromatic triisocyanate, and aromatic tetraisocyanate. Specific examples of the aromatic polyisocyanate include, for example, m-phenylene diisocyanate, p-phenylene diisocyanate, 4,4'-diphenyl diisocyanate, 1,5-naphthalene diisocyanate, 2,4'- or 4,4'-diphenylmethane diisocyanate, or a mixture thereof, 2,4- or 2,6-tolylene diisocyanate or a mixture thereof, triphenylmethane-4,4',4"-triisocyanate, and 4,4'-diphenylmethane-2,2',5,5'-tetraisocyanate. These may be used singly or in combination of two or more thereof.

Examples of the derivative of the polyisocyanate include various derivatives such as a dimer, trimer, biuret, allophanate, carbodiimide, urethodione, urethoimine, isocyanurate, and iminooxadiazinedione of the aforementioned polyisocyanate compounds. These may be used singly or in combination of two or more thereof.

These polyisocyanates can be used singly or in combination of two or more thereof.

As the polyisocyanate compound, a blocked polyisocyanate compound (blocked isocyanate), which is a compound obtained by blocking isocyanate groups of the polyisocyanate compound with a blocking agent, is preferably used. The blocked polyisocyanate compound is preferably used because it is relatively stable even in solution and can be used in the same solution as solution of the repellent.

The blocking agent is an agent that blocks free isocyanate groups. The blocked polyisocyanate compound, for example, can be heated 100°C or higher, for example, 130°C or higher to regenerate isocyanate groups, facilitating a reaction with hydroxyl groups. Examples of the blocking agent include, for example, a phenolic compound, lactam-based compound, aliphatic alcohol-based compound, and oxime-based compound. The polyisocyanate compound may be used singly or in combination of two or more thereof.

The epoxy compound is a compound having an epoxy group. Examples of the epoxy compound include epoxy compounds having a polyoxyalkylene group, such as a polyglycerol polyglycidyl ether and a polypropylene glycol diglycidyl ether; as well as a sorbitol polyglycidyl ether.

The chloromethyl group-containing compound is a compound having a chloromethyl group. Examples of the chloromethyl group-containing compound include, for example, a chloromethyl polystyrene.

The carboxyl group-containing compound is a compound having a carboxyl group. Examples of the carboxyl group-containing compound include, for example, a (poly)acrylic acid, and a (poly)methacrylic acid.

Specific examples of the ketone group-containing compound include, for example, a (poly)diacetone acrylamide, and diacetone alcohol.

Specific examples of the hydrazide compound include, for example, hydrazine, a carbohydrazide, and adipic acid hydrazide.

Specific examples of the melamine compound include, for example, a melamine resin and a methyl etherified melamine resin.

### [Amount of Curing Agent]

The amount of the curing agent may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, and 5 parts by weight or less.

### {Other Component}

The repellent may contain a component other than the aforementioned components. Examples of the other components include, for example, polysaccharides, a paper strengthening agent, an agglomerating agent, a yield improver, a coagulant, a binder resin, an anti-slip agent, a sizing agent, a paper strengthening agent, a filler, an antistatic agent, an antiseptic agent, an ultraviolet absorber, an antibacterial agent, a deodorant, and a fragrance. These may be used singly or in combination of two or more thereof.

In addition to the above components, as other components, for example, other water-repellent and/or oil-repellent agents, a dispersant, a texture modifier, a softening agent, a flame retarder, a coating material fixing agent, a wrinkle-resistant agent, a drying rate adjuster, a cross-linking agent, a film formation agent, a compatibilizer, an antifreezing agent, a viscosity adjuster, an ultraviolet absorber, an antioxidant, a pH adjuster, an insect repellent, an antifoaming agent, an anti-shrinkage agent, a laundry wrinkle-resistant agent, a shape retention agent, a drape retention agent, an ironing improving agent, a brightening agent, a whitening agent, fabric softening clay, a migration-proofing agent such as a polyvinylpyrrolidone, a polymer dispersant, a soil release agent, a scum dispersant, a fluorescent brightening agent such as 4,4-bis(2-sulfostyryl)biphenyldisodium (Tinopal CBS-X manufactured by Ciba Specialty Chemicals Plc), a dye fixing agent, an anti-color fading agent such as 1,4-bis(3-aminopropyl)piperazine, a stain removing agent, enzymes such as cellulase, amylase, protease, lipase, and keratinase as fiber surface modifiers, a foam inhibitor, and silk protein powder that can impart texture and functions of silk such as moisture absorption and release properties, and surface modified products or emulsified dispersions thereof (for example, K-50, K-30, K-10, A-705, S-702, L-710, FP series (Idemitsu Petrochemical Co., Ltd.), hydrolyzed silk liquid (Jomo), SILKGEN G Soluble S (ICHIMARU PHARCOS Co., Ltd.)), an antifouling agent (for example, a nonionic polymer compound composed of an alkylene terephthalate and/or an alkylene isophthalate units and a polyoxyalkylene unit (for example, FR627 manufactured by GOO CHEMICAL CO., LTD.), SRC-1 manufactured by Clariant (Japan), K. K.), can be compounded. These may be used singly or in combination of two or more thereof.

### [Amount of Other Component]

Each amount or the total amount of other components may be 0.1 parts by weight or more, 1 part by weight or more, 3 parts by weight or more, 5 parts by weight or more, 10 parts by weight or more, 15 parts by weight or more, 20 parts by weight or more, 50 parts by weight or more, 75 parts by weight or more, or 100 parts by weight or more, relative to 100 parts by weight of the wax, and may be 500 parts by weight or less, 300 parts by weight or less, 200 parts by weight or less, 100 parts by weight or less, 50 parts by weight or less, 40 parts by weight or less, 30 parts by weight or less, 20 parts by weight or less, 10 parts by weight or less, or 5 parts by weight or less.

### <Method for producing pulp composition/ pulp product>

The pulp composition of the present disclosure may be obtained by treating a pulp substrate with a repellent containing a wax.

A pulp product may be obtained by subjecting the resulting pulp composition to processing such as drying, heating and forming according to need.

The repellent in the present disclosure can be applied to a pulp substrate as a treatment agent (particularly a surface-treating agent) by a conventionally known method. The treatment method may be a method for dispersing the repellent in the present disclosure in an organic solvent or water, if necessary, to dilute it and allowing it to adhere to an inside of a pulp substrate and/or on a surface thereof and drying by a known method such as dip coating, spray coating, and foam coating. The dilution factor, which may be changed depending on the concentration and the purpose of use of the repellent, may be 3 to 2,000 times, and for example, 10 to 100 times. After drying, a pulp product to which a solid component of the repellent has been adhered, is obtained. If necessary, the repellent of the present disclosure may be applied in combination with a suitable cross-linking agent, and curing may be carried out.

The repellent can be applied to a pulp substrate by any of methods known for treating a pulp substrate with liquid. The pulp substrate may be immersed in the repellent, the pulp substrate and the repellent may be mixed, or solution may be adhered or sprayed onto the pulp substrate. The treated pulp substrate is preferably dried and cured by heating in order to develop liquid-repellency. The heating temperature may be, for example, 100°C to 200°C, 100°C to 170°C, or 100°C to 120°C. In the present disclosure, the heating time may be 5 seconds to 60 minutes, for example, 30 seconds to 3 minutes.

As the method for treating a pulp substrate, an internal addition treatment method in which repellent is added to a pulp substrate before papermaking (e.g., in the form of pulp slurry), or an external addition treatment method in which repellent is applied to a pulp substrate after papermaking (e.g., a pulp product), can be employed. Examples of internal addition treatment methods include mixing and dipping, and the internal addition treatment method may include a step of adding a repellent to pulp slurry and mixing it with stirring. Examples of external addition treatment methods include spraying, coating, dipping and foam coating and more specifically a pound-type two-roll size press, a gate roll type size press and a rod metering type size press. The treatment may be external addition treatment or internal addition treatment. For example, when the pulp substrate is paper, the repellent may be applied to paper, or solution may be adhered or sprayed onto paper, or the repellent may be mixed with pulp slurry before papermaking to perform treatment. When the pulp substrate is a fiber material, examples of treatment methods include padding treatment, dip treatment, spray treatment, and coating treatment. Examples of padding treatment include the method involving using the padding apparatus as described on pages 396 to 397 of Seni Sensyoku Kako Jiten (in Japanese; Fiber-dyeing process dictionary) (published by THE NIKKAN KOGYO SHIMBUN, LTD., 1963) and pages 256 to 260 of Irozome Kagaku (in Japanese; dyeing chemistry) III (published by Jikkyo Shuppan Co., Ltd., 1975). Examples of the coating treatment include the method involving using a coating machine as described on pages 473 to 477 of Sensyoku Shiage Kiki Soran (in Japanese; Comprehensive guide to dyeing and finishing machines) (published by Fiber Japan CO., LTD., 1981). Examples of the dip treatment include the method involving using a batch type dyeing machine as described on pages 196 to 247 of Sensyoku Shiage Kiki Soran (in Japanese; Comprehensive guide to dyeing and finishing machines) (published by Fiber Japan CO., LTD., 1981), and for example, a jet dyeing machine, air flow dyeing machine, drum dyeing machine, wince dyeing machine, washer dyeing machine, and cheese dyeing machine can be used. Examples of the spray treatment include a method involving using an air spray that nebulizes and sprays a treatment liquid by compressed air, or an air spray by hydraulic pressure nebulization system.

The method of treatment may be internal addition treatment in which a repellent is added to pulp slurry before papermaking. The internal addition treatment may include, but is not limited to, one or more of a step of adding the repellent to pulp slurry and mixing it with stirring; a step of sucking and dehydrating the pulp composition prepared in the step through a net-like body of predetermined shape and depositing the pulp composition then to form a pulp formed article intermediate; and a step of molding and drying the pulp formed article intermediate by using a heated molding mold to obtain a pulp formed article. After having been lightly dried at room temperature or elevated temperature, the treated paper may be optionally subjected to heat treatment, depending on the nature of the paper. The temperature of the heat treatment may be 150°C or higher, 180°C or higher, or 210°C or higher, and may be 300°C or lower, 250°C or lower, or 200°C or lower, particularly 80°C to 180°C. Carrying out the heat treatment in such a temperature range enables exhibiting, for example, excellent oil resistance and water resistance. The pulp substrate which has undergone internal addition treatment may be subjected to external addition treatment to be treated with the repellent, allowing another wax or repellent to be adhered to the surface.

The treatment method may be an external addition treatment in which repellent is applied to a pulp substrate after papermaking. The size press used in external addition treatment may be classified depending on the coating method as follows. One coating method involves supplying a coating liquid (size liquid) to a nip portion formed by passing paper between two rubber rolls, creating a pool of the coating liquid called a pond, and allowing the paper to pass through this pool to coat both sides of the paper with the size liquid, which is a method employed for a so-called pound-type two-roll size press. Another coating method is a method used for a gate roll type size press in which a size liquid is applied by a surface transfer type, and a rod metering type size press. In the pound-type two-roll size press, the size liquid easily penetrates into an inside of paper, and in the surface transfer type, a size liquid component is likely to stay on a surface of the paper. In the surface transfer type, a coating layer is likely to stay on a surface of paper more than in the pound-type two-roll size press, and the amount of coating layer formed on the surface is more than in the pound-type two-roll size press. In the present disclosure, even in the case of using the former pound-type two-roll size press, performance can be imparted to paper. After having been lightly dried at room temperature or elevated temperature, the paper treated in such a manner is arbitrarily accompanied by heat treatment that can have a temperature range of up to 300°C, for example up to 200°C, and particularly the temperature range of 80°C to 180°C, depending on the nature of the paper, as a result of which excellent oil resistance, water resistance, and the like can be exhibited.

Specific examples of the paper products include, for example, paper, a paper container, a pulp formed article, a food packaging material, a food container, gypsum liner board base paper, coated base paper, medium-quality paper, a general liner and core, neutral pure white roll paper, a neutral liner, a rust-proof liner, and metal pasted paper, kraft paper, neutral printing writing paper, neutral coated base paper, neutral PPC paper, neutral thermal paper, neutral pressure-sensitive base paper, neutral inkjet paper and neutral information paper. Preferred examples of pulp products include a food packaging material and a food container, and in particular, a pulp formed article for food contact.

Embodiments have been described above, but it will be understood that various modifications can be made to embodiments and details without departing from the spirit and the scope of the claims.

### Examples

Hereinafter, the present disclosure will be described in detail with reference to Examples, but the present disclosure is not limited to these Examples.

### <Test Method>

The test procedures are as follows.

### [Volume abundance ratio and median diameter (D50) of particle]

The volume abundance ratio of particles with a size of 100 µm or larger, the volume abundance ratio of particles with a size of 10 µm or larger and the median diameter (D50) of the wax and the aqueous dispersion were calculated from the volume-based frequency distribution (volume distribution) obtained by the measurement using a laser diffraction/scattering apparatus.

### [Preparation of paraffin wax dispersion]

2 g of paraffin wax (melting point 69.8°C), 0.2 g of polyethylene oxide alkyl ether (in which alkyl has 6 to 16 carbon atoms, HLB: 7) and 17.8 g of water were mixed to give an aqueous dispersion. The aqueous dispersion was heated to 85°C and then treated by a ultrasonic homogenizer for 20 minutes to give a water-dispersible repellent. The resulting water-dispersible repellent had the following properties.
Median diameter D50: 0.8 µm
Volume abundance ratio of particle with a size of 100 µm or larger: 0%
Volume abundance ratio of particle with a size of 10 µm or larger: 12%
Charge density: 20 µeq/g

### [Preparation of microcrystalline wax dispersion]

Microcrystalline wax (melting point 79°C) was pulverized to 1 mm or less in a mortar and subjected to a dry pulverization treatment by a jet mill to give a powder of the microcrystalline wax. The particle size of the powder of the microcrystalline wax was measured using a laser diffraction/scattering apparatus, and as a result the powder had a median diameter D50 of 0.99 µm. 2 g of the resulting powder of microcrystalline wax, 0.2 g of polyethylene oxide alkyl ether (in which alkyl has 6 to 16 carbon atoms, HLB: 7) and 17.8 g of water were mixed to give a water-dispersible repellent. The resulting water-dispersible repellent had the following properties.
Median diameter D50: 0.95 µm
Volume abundance ratio of particle with a size of 100 µm or larger: 0%
Volume abundance ratio of particle with a size of 10 µm or larger: 25%
Charge density: 2 µeq/g

### [Preparation of pulp mold]

Pulp mold was formed using an automatic mold molding machine. In the lower part thereof, a net-like body was arranged on a pulp mold molding mold made of metal with many suction holes, a metal tank was arranged in the upper part, and a mixture of pulp slurry and the water-dispersible repellent (a pulp composition) was charged in the upper metal tank. From the opposite side of the pulp mold molding mold to the side where the net-like body was arranged, the pulp composition was suctioned and dehydrated through the pulp mold molding mold and the net-like body by a vacuum pump, and solids (pulp, etc.) contained in the pulp composition were allowed to deposit on the net-like body to obtain a pulp mold intermediate. Next, the resulting pulp mold intermediate was dried by applying pressure of 0.05 to 5 MPa thereto from the tops and bottoms of male and female molding molds made of metal, which have been heated to 60 to 250°C. Thus, a pulp mold product formed into the shape of a container was produced.

### [Oil-resistance test]

After pouring 100 ml of corn oil at 50°C into the pulp mold and allowing it to stand at room temperature for 45 minutes, the corn oil was removed from the pulp mold, and the degree of staining in the pulp mold was evaluated. The evaluation scores were set as follows according to the degree of staining.
5: No stains inside the pulp mold.
4: Stains inside the pulp mold. No stains on the backside.
3: Stains the inside the pulp mold. Slight stain bleed out on the backside.
2: Stains inside the pulp mold. The area of stain bleed out to the backside is less than 50% of the total area.
1: Stains inside the pulp mold. The area of stain bleed out to the backside is 50% or more and less than 100% of the total area.
0: Stains over the backside.

### [Water resistance test]

After pouring 100 ml of evaluation liquid (water) at 100°C into the pulp mold and allowing it to stand at room temperature for 30 minutes, the evaluation liquid was removed from the pulp mold, and the degree of staining in the pulp mold was evaluated. Evaluation scores were set as follows depending on the degree of staining.
5: No stains inside the pulp mold.
4: Stains inside the pulp mold. No stains on the backside.
3: Stains inside the pulp mold. Slight stain bleed out on the backside.
2: Stains inside the pulp mold. The area of stain bleed out to the backside is less than 50% of the total area.
1: Stains inside the pulp mold. The area of stain bleed out to the backside is 50% or more and less than 100% of the total area.
0: Stain bleed out over the backside.

### <Example 1>

An aqueous pulp slurry with a concentration of 0.5% by weight containing 75% of wood pulp and 25% of bagasse pulp based on the total amount of pulp was prepared. The water-dispersible repellent was added thereto so that the ratio of the dispersion was 3% by weight in terms of solid content, relative to pulp, to prepare a pulp composition. The pulp composition was charged into an automatic mold molding machine to prepare a pulp mold. The pulp mold prepared was subjected to the oil-resistance test and the water-resistance test, which scored 4 points in the oil-resistance test and 1 point in the water-resistance test. The results are shown in Table 1.

### <Example 2>

An aqueous pulp slurry with a concentration of 0.5% by weight containing 100% of bagasse pulp based on the total amount of pulp was prepared. The water-dispersible repellent was added thereto so that the ratio of the dispersion was 3% by weight in terms of solid content, relative to pulp, to prepare a pulp composition. The pulp composition was charged into an automatic mold molding machine to prepare a pulp mold. The pulp mold prepared was subjected to the oil-resistance test and the water-resistance test, which scored 4 points in the oil-resistance test and 1 point in the water-resistance test. The results are shown in Table 1.

### <Example 3>

When the pulp composition was prepared, the water-dispersible repellent was added to pulp slurry so that the ratio of the repellent was 1% by weight in terms of solid content, relative to pulp. Then pulp mold was prepared in the same manner as in Example 1. The pulp mold prepared was subjected to the oil-resistance test and the water-resistance test, which scored 4 points in the oil-resistance test and 1 point in the water-resistance test. The results are shown in Table 1.

### <Example 4>

Pulp mold was prepared in the same manner as in Example 1 except for adding 0.45% by weight of AKD (alkyl ketene dimer) based on pulp when the pulp composition was prepared. The pulp mold prepared was subjected to the oil-resistance test and the water-resistance test, which scored 4 points in the oil-resistance test and 5 points in the water-resistance test. The results are shown in Table 1.

### <Example 5>

Pulp mold was prepared in the same manner as in Example 1 except for adding 0.1% by weight of a rosin sizing agent based on pulp when the pulp composition was prepared. The pulp mold prepared was subjected to the oil-resistance test and the water-resistance test, which scored 4 points in the oil-resistance test and 5 points in the water-resistance test. The results are shown in Table 1.

### <Example 6>

Pulp mold was prepared in the same manner as in Example 1 except for adding 1% by weight of cationic starch based on pulp when the pulp composition was prepared. The pulp mold prepared was subjected to the oil-resistance test and the water-resistance test, which scored 4 points in the oil-resistance test and 2 points in the water-resistance test. The results are shown in Table 1.

### <Example 7>

Pulp mold was prepared in the same manner as in Example 1 except for adding 0.1% by weight of polyacrylamide based on pulp when the pulp composition was prepared. The pulp mold prepared was subjected to the oil-resistance test and the water-resistance test, which scored 4 points in the oil-resistance test and 2 points in the water-resistance test. The results are shown in Table 1.

### <Example 8>

Pulp mold was prepared in the same manner as in Example 1 except for using microcrystalline wax instead of paraffin wax. The pulp mold prepared was subjected to the oil-resistance test and the water-resistance test, which scored 4 points in the oil-resistance test and 2 points in the water-resistance test. The results are shown in Table 1.

### <Comparative Example 1>

An aqueous pulp slurry with a concentration of 0.5% by weight containing 100% of wood pulp based on the total amount of pulp was prepared, and pulp mold was prepared in the same manner as in Example 1. The pulp mold prepared was subjected to the oil-resistance test and the water-resistance test, which scored 2 points in the oil-resistance test and 1 point in the water-resistance test.

### <Comparative Example 2>

An aqueous pulp slurry with a concentration of 0.5% by weight containing 25% of bagasse pulp and 75% of wood pulp based on the total amount of pulp was prepared. The pulp slurry was charged into an automatic mold molding machine to prepare a pulp mold. The pulp mold prepared was subjected to the oil-resistance test and the water-resistance test, both of which scored 0 points.

### <Comparative Example 3>

An aqueous pulp slurry with a concentration of 0.5% by weight containing 100% of bagasse pulp based on the total amount of pulp was prepared. The pulp slurry was charged into an automatic mold molding machine to prepare a pulp mold. The pulp mold prepared was subjected to the oil-resistance test and the water-resistance test, both of which scored 0 points.

The results are summarized in the following table.

**[Table 1]**

| | Repellent | Bagasse pulp (%) | Wood pulp (%) | Amount of repellent added (%) | Combination chemical | Oil resistance | Water resistance |
|---|---|---|---|---|---|---|---|
| Example 1 | Paraffin wax | 25 | 75 | 3 | - | 4 | 1 |
| Example 2 | Paraffin wax | 100 | 0 | 3 | - | 5 | 1 |
| Example 3 | Paraffin wax | 100 | 0 | 1 | - | 4 | 1 |
| Example 4 | Paraffin wax | 25 | 75 | 3 | AKD | 4 | 5 |
| Example 5 | Paraffin wax | 25 | 75 | 3 | Rosin sizing agent | 4 | 5 |
| Example 6 | Paraffin wax | 25 | 75 | 3 | Cationic starch | 4 | 2 |
| Example 7 | Paraffin wax | 25 | 75 | 3 | PAM | 4 | 2 |
| Example 8 | Microcrystal line wax | 25 | 75 | 3 | - | 5 | 1 |
| Comparative Example 1 | Paraffin wax | 0 | 100 | 3 | - | 2 | 1 |
| Comparative Example 2 | - | 25 | 75 | 0 | - | 0 | 0 |
| Comparative Example 3 | - | 100 | 0 | 0 | - | 0 | 0 |

## Claims

1. A pulp composition comprising a wax and a pulp substrate,
wherein
the wax is a hydrocarbon wax, and
the pulp substrate comprises bagasse pulp.

2. The pulp composition according to claim 1, wherein the wax is at least one selected from the group consisting of paraffin wax and microcrystalline wax.

3. The pulp composition according to claim 1 or 2, wherein the wax has a melting point of 40°C or more and 120°C or less.

4. The pulp composition according to any one of claims 1 to 3, wherein an amount of the wax is 0.5% by weight or more and 25% by weight or less based on the pulp substrate.

5. The pulp composition according to any one of claims 1 to 4, wherein an amount of the bagasse pulp is 20% by weight or more and 100% by weight or less in the pulp substrate.

6. The pulp composition according to any one of claims 1 to 5, wherein the pulp composition comprises a dispersant.

7. The pulp composition according to any one of claims 1 to 6, wherein the pulp composition comprises a combination chemical for paper.

8. The pulp composition according to any one of claims 1 to 7, wherein the pulp composition comprises at least one selected from the group consisting of a sizing agent and a paper strength agent.

9. The pulp composition according to any one of claims 1 to 8, wherein the pulp composition comprises aluminum sulfate.

10. A pulp formed article formed from the pulp composition according to any one of claims 1 to 9.

11. The pulp formed article according to claim 10, which is for food contact.

12. A method for producing a pulp composition, comprising treating a pulp substrate with a repellent comprising a wax,
wherein
the wax is a hydrocarbon wax, and
the pulp substrate comprises bagasse pulp.

13. The method for producing a pulp composition according to claim 12, wherein the wax is at least one selected from the group consisting of paraffin wax and microcrystalline wax.
